

Patented July 28, 1925.

1,547,815

# UNITED STATES PATENT OFFICE.

DEAN M. JACKMAN, OF KENVIL, AND FREDRICH OLSEN, OF DOVER, NEW JERSEY.

## EXPLOSIVE COMPOSITION.

No Drawing.

Application filed October 30, 1923. Serial No. 671,752.

(GRANTED UNDER THE ACT OF MARCH 3, 1883; 22 STAT. L. 625.)

To all whom it may concern:

Be it known that we, DEAN M. JACKMAN and FREDRICH OLSEN, citizens of the United States, and residents of Kenvil, county of Morris, and State of New Jersey, and Dover, county of Morris, and State of New Jersey, respectively, invented an Improvement in Explosive Compositions, of which the following is a specification.

10 The invention described herein may be used by the Government, or any of its officers or employees in prosecution of work for the Government, or by any other person in the United States, without payment to me of any royalty thereon, in accordance with the act of March 3, 1883.

The subject matter of this invention is an explosive composition.

20 The primary object of our invention is the provision of an explosive which will generate great power at the moment of explosion yet will be sufficiently insensitive to withstand all ordinary shocks.

25 A further object is the establishment of a method by which such an explosive may be manufactured.

With the foregoing and other objects in view my invention resides in the novel arrangement and combination of ingredients 30 and in the details of preparation herein-after described and claimed, it being understood that changes in the precise embodiment of the invention herein disclosed may be made within the scope of what is claimed 35 without departing from the spirit of the invention.

Experiments conducted with the phenyl and tolyl derivatives of guanidine and their salts show that, by nitrating these derivatives of guanidine or their salts, compounds 40 may be obtained which will have many desirable explosive properties. The present invention then is intended to cover the use of these derivatives and the process by 45 which they may be prepared.

Up to the present time the most satisfactory substance treated has been diphenyl guanidine. Further experiments, however, with this and other phenyl and tolyl derivatives 50 is now being conducted and it is by no means intended to limit this invention to the preparation of an explosive from this one substance alone. The process, however,

by which this substance is treated is typical 55 of the methods pursued in the treatment of other phenyl and tolyl derivatives of guanidine and their salts and is given as explanatory and illustrative of the procedure which is part of the subject matter of this 60 invention.

Under this process diphenyl guanidine (symmetrical) is nitrated by treating the guanidine with a sufficient amount of a mixture of nitric and sulphuric acids. After a sufficient interval the whole is then poured 65 into a large volume of water. A yellow substance separates from the liquid; the precipitate thus formed is recovered by filtration.

The composition of this substance has not 70 yet been fully determined. It is probably not a single compound as it has so far been obtained but a mixture of isomers or even more distantly related compounds. The substance probably consists essentially of 75 hexanitro-diphenyl guanidine:



or a diphenyl guanidine having 7 or 8 hydrogen atoms replaced by nitro groups as in the combination:



The substance as already obtained, however, has been found to be slightly less sensitive than tetryl and about 1/3 more powerful which makes it a highly valuable explosive composition.

The method pursued in treating the diphenyl guanidine has been followed successfully in the treatment of other phenyl and tolyl derivative of guanidine and their 105 salts and both the use of the substances

formed by the nitration of these derivatives and the process pursued in their nitration is considered novel.

We claim:

5. 1. A new explosive embodying a nitro-diphenyl guanidine.
2. A new explosive embodying a nitro-phenyl derivative of guanidine.
3. A new explosive embodying a nitro-tolyl derivative of guanidine.
10. 4. A new explosive embodying a nitro-aromatic derivative of guanidine.
5. The process of preparing an explosive which includes treating diphenyl guanidine with nitric and sulphuric acids, pouring the 15 whole into water and separating the precipitate thus formed.
6. The process of preparing an explosive which includes treating a phenyl derivative 20 of guanidine with acids to nitrate the same,

pouring the whole into water and separating the precipitate thus formed.

7. The process of preparing an explosive which includes treating a tolyl derivative of guanidine with acids to nitrate the same, 25 pouring the whole into water and separating the precipitate thus formed.

8. The process of preparing an explosive which includes treating an aromatic derivative of guanidine with nitric and sulphuric acids, 30 pouring the whole into water and separating the precipitate thus formed.

9. The process of preparing an explosive which includes treating an aromatic derivative of guanidine with acids to nitrate the 35 same, pouring the whole into water and separating the precipitate thus formed.

DEAN M. JACKMAN.  
FREDRICH OLSEN.